

Sept. 7, 1926.

1,599,136

W. H. KOBBE

RAILWAY TIE

Filed Dec. 21, 1925

3 Sheets-Sheet 1



Sept. 7, 1926.

1,599,136

W. H. KOBBE

RAILWAY TIE

Filed Dec. 21, 1925

3 Sheets-Sheet 2



Fig. 2

PER CENT CEMENT

INVENTOR

William H. Kobbé

BY

Connie, Davis, Marvin and Edwards  
his ATTORNEYS

Sept. 7, 1926.

1,599,136

W. H. KOBBE

RAILWAY TIE

Filed Dec. 21, 1925

3 Sheets-Sheet 3



Fig. 3

INVENTOR

William H. Kobbé

BY

Perme, Davis, Marion & Edward  
his ATTORNEYS

## UNITED STATES PATENT OFFICE.

WILLIAM HOFFMAN KOBBE, OF NEW YORK, N. Y., ASSIGNOR TO TEXAS GULF SULPHUR COMPANY, OF BAY CITY, TEXAS, A CORPORATION OF TEXAS.

## RAILWAY TIE.

Application filed December 21, 1925. Serial No. 76,587.

The present invention relates to railway ties or sleepers used in railway construction, and has for its object the provision of an improved railway tie.

5 Although wooden ties have been used almost exclusively since the beginning of railways in this country, there has been a gradual change in the kind of wood used. Formerly only the best grade of oak was employed but with the advancing cost of wood, and the scarcity of oak, many other species are now being utilized. Wood preservation has proved advantageous and southern pine, cypress and other species are now being made 10 into ties and treated with creosote and other materials. However, the increasing scarcity of the various woods now available that are suitable for ties makes the necessity for substitute materials more and more apparent.

15 20 Wood possesses no particular quality which makes it superior to other materials, but it is cheaper, and heretofore no substitute has been found which will successfully compete economically with a wooden tie, particularly when treated in accordance with present day practice.

A resilient road bed, such as is obtained by the use of wooden ties, was at one time thought essential but the advocates of the 30 rigid type of track construction employing concrete or metal ties have proved that the advantages of the resilient tie are outweighed by the many advantages of the rigid type of construction. Concrete or 35 metal ties would therefore come into more general use were it not for the fact that the life of a concrete or steel tie as now made is not sufficiently in excess of that of a treated wooden tie of high quality to compensate 40 for the difference in first cost.

An idea of the industrial importance of the problem is indicated by the following figures which represent the approximate tie requirements per year of various countries:

|               |            |
|---------------|------------|
| 45 Germany    | 5,600,000  |
| Great Britain | 5,600,000  |
| France        | 5,400,000  |
| Italy         | 1,800,000  |
| Switzerland   | 800,000    |
| 50 Holland    | 280,000    |
| Spain         | 1,500,000  |
| United States | 36,000,000 |

The improved railway tie of my present invention costs somewhat more than either

wood or concrete but the improved properties which it possesses more than justify the increased first cost. I have discovered that sulphur, when appropriately associated therewith imparts certain qualities to railway ties which renders ties made of many substitute materials far superior to wooden ties as commonly made and treated, and in addition, when associated with railway ties of inferior species of wood makes them the equal of ties made of hard, durable species. 65 Thus, according to my invention, woods which have heretofore been unsuited for use as railway ties may now be used.

It is to be understood, moreover, that the term "substitute materials" is intended to 70 include, not only concrete, but any substitute for wooden railway ties, and the invention hence involves the provision of a sulphur-containing railway tie.

In carrying out the invention, the railway tie which, let us say, is constructed in this instance of wood, is immersed in and held beneath the surface of a bath of molten sulphur which is maintained at a temperature preferably of about 140 to 150° C. for the 75 first 5 or 6 hours, or until the evidence of moisture has disappeared. It is then desirable to allow the temperature of the bath to drop to about 120 or 125° C. for the remainder of the time or 4 to 5 hours, when 80 the tie is removed. The extent of penetration is generally evidenced by the buoyancy of the tie in the sulphur bath and complete cessation of bubbling. A fully impregnated white pine tie will expose only about one-fifth of its volume above the surface of the 85 sulphur, and will of course sink in water.

The period of immersion depends upon many factors, but in general I leave the ties made of various woods in the bath for not 90 less than 10 or 12 hours and in some cases double this time has little effect upon the total quantity absorbed. A readily impregnated tie may require only 4 or 5 hours, but in all investigations to date an effort has 95 been made to secure maximum impregnation irrespective of the time element in order to determine just what woods may be treated by the simple open tank immersion method without the application of vacuum or pressure, and the portion of the tree best adapted 100 for this method of impregnation.

In my investigations, white pine, sugar or

western white pine, red and white palmetto, so-called soft and hard California redwood, poplar, cypress, white wood (*Liriodendron tulipifera*), hard maple, beech, birch, red oak, white spruce, cedar and other species have been impregnated with sulphur. These include the various types of woody growth such as hardwood or broadleaved species, soft woods or conifers, and the palms.

- 10 The use of vacuum and/or pressure expedites the impregnation process, but in some cases there is not sufficient increase in the quantity of sulphur entering the wood to justify the expense of its employment.
- 15 Certain species of wood absorb approximately as much sulphur by the open tank treatment as would enter the wood under vacuum and pressure. Certain species which are very resistant to impregnation by open tank treatment are equally difficult to impregnate with vacuum and pressure.

In order to secure the most thorough impregnation it is important that the wood be seasoned or properly dried before the ties 25 are given the sulphur treatment because the presence of moisture inhibits penetration of sulphur and when in excess, prevents the entry of practically any sulphur. This may be explained by the fact that it is difficult 30 for the sulphur to enter the tracheids, pores or resin ducts while moisture is being driven off in the form of steam, and in addition, the conversion of water into steam requires a certain amount of heat and has a tendency 35 to lower the temperature of the woody mass, with the constant cooling of the molten sulphur in immediate contact with the wood.

I have found that dry white pine, especially the sapwood, absorbs several times its 40 own weight of sulphur and when impregnated, consists of as much as 60% to 70% by weight of sulphur based upon the final weight of the treated wood. California redwood absorbs approximately its own 45 weight of sulphur, while Florida palmetto absorbs about the same as white pine, or from 60% to 70%, but requires a much longer period of immersion. The other species of wood mentioned in this specification 50 absorb anywhere from about 5% or 6% up to about 50% or more sulphur, depending upon the conditions and structure of the wood.

The effect of the association of sulphur 55 with the wooden railway tie is to indurate and strengthen it. Under compression parallel to the grain untreated pine withstood under test a maximum load of 3,500 pounds per square inch, whereas pine impregnated 60 with sulphur by the open tank method for a period of about 12 hours, or in other words, impregnated to the maximum extent, required 5,800 pounds per square inch to bring 65 about the failure. The sulphur treated wooden tie is also much more resistant to

impact and is several times harder than the untreated. For example, if the hardness of untreated hemlock is taken as 100, sulphur treated hemlock was found under test to have a hardness of from about 300 to 350. 70

As is well known, California redwood will last almost indefinitely in the ground, but it cannot be used for railroad ties under heavy traffic because the rails, either with or without tie plates, cut into and destroy the tie 75 long before the center portion has deteriorated in any way. By treating the tie with sulphur according to my invention it is possible to so indurate or harden the wood as to admirably adapt it for use as a railway 80 tie. Such a tie may be completely impregnated with sulphur if desired but a partial impregnation sufficient to harden the wood in the region of the surface of the tie, say for example to a depth of about 1" is sufficient. This hardening of the surface greatly reduces the rate of cutting by the rails and a tie is thus produced which is extraordinarily 85 serviceable. If desired, only the ends or the wearing surfaces of the tie need be impregnated with sulphur.

Other woods are rendered, by the process of the invention much more durable for use as railway ties because of the preservative qualities imparted by the sulphur as well as 90 the increase in hardness and strength resulting from the sulphur treatment. In order to bring about wood rot the presence of heat, moisture and oxygen are necessary, and sulphur excludes at least two of these agencies. 95 In other words, the sulphur preserves the wood physically rather than by chemical means and isolates it from the action of wood rot fungi. Therefore, although not in itself toxic, sulphur acts as a preservative 100 of the wood in that it excludes and prevents the entry and action of the destructive agencies.

The extent of impregnation desirable will 105 also depend upon what physical properties it is desired to improve. Thus if merely an increase in resistance to mechanical abrasion and wear is desired, a mere surface impregnation is all that is required. On the other hand, although the surface impregnation 110 will increase the strength of the tie to a certain extent depending upon the depth to which it is carried, if a maximum increase 115 in strength is desired, as much sulphur as is possible should be allowed to congeal within the pores of the tie.

Another advantage in the sulphur treated tie is to be found in the fact that it will hold spikes much better than the untreated ties. A practical consideration in connection with the invention is the fact that the impregnation of the ties with sulphur may be carried out in the usual creosoting cylinders now extensively employed for injecting creosote oil into railway ties. 120

Sulphur being an insoluble solid at ordinary temperatures, the effect of my treatment is different from that brought about by the use of any other impregnant. Creosote does not change its form after entering the wood, nor do the various waxes such as Montan wax, or the metallic salts similarly employed unless such salts enter the wood in the form of a solution. On the other hand, my treatment injects an elemental fluid into the wood which becomes a crystalline solid and this change is so rapid that the surface pores are almost immediately closed through solidification of the sulphur and "kick-back" such as occurs with other materials, is prevented. For example, when creosote oil is forced into wood under pressure, and this pressure is removed, a portion of the oil exudes from the wood because there is nothing to counteract the internal pressures. In my process, the rapid solidification of the sulphur on the surface and particularly at the ends of the treated wood, immediately seals the pores and prevents the loss of the molten sulphur contained within the woody structure.

The sulphur treatment of the invention is particularly applicable to concrete ties which heretofore have not been sufficiently strong to withstand traffic conditions, even though heavily reinforced with metal.

Ultimate failure in an untreated concrete tie is brought about through mechanical and chemical agencies of a destructive nature. The impact of the rail under traffic, gradual movement and creeping of the rail and rail fastenings and the absorption and freezing of water within the tie structure are the more important destructive agencies of a mechanical nature. In addition, chemical processes play a part in the destruction of an ordinary concrete tie. Tie plates, rail fastenings and the reinforcing metal oxidize and occupy an increased volume which is destructive to the ties. Corrosive soils or ballast material which contain sulphates are also very destructive to ordinary concrete.

I have discovered that by impregnating concrete ties with sulphur, both the tensile and compressive strength are increased from five to ten times and such ties are highly resistant to the various destructive agencies mentioned. The sulphur-containing ties are so much stronger than an ordinary concrete tie that in many cases reinforcement is found to be unnecessary, but it may be included without any ill effect since the sulphur largely protects the metal from corrosion.

In treating concrete railway ties in accordance with the present invention, the ties after having been moulded from a suitable concrete mixture such for example as

material such as crushed rock and/or sand and/or gravel, are immersed in a bath of molten sulphur which is maintained at a temperature of from 140 to 150° C. for a number of hours, as in the case of the impregnation of wood. After the moisture appears to have been driven off, the temperature of the bath is then reduced to in the neighborhood of 120 to 125° C. for a further number of hours.

The period of immersion at the higher temperature as well as the total period of immersion depends, as in the case of the impregnation of wood, upon many factors, such for example as the penetrability of the concrete mixture, and the extent of impregnation desired. If a material increase in strength is looked for, the ties should be impregnated until the sulphur has penetrated to a considerable depth, if not throughout the entire mass of the concrete, but if it is only desired to render the ties resistant to the destructive agencies to which they are subjected in service, a relatively shallow impregnation, say for example from  $\frac{1}{2}$ " to 1" is all that is necessary. This partial impregnation is obtained in a correspondingly shorter length of time. The concrete ties may be impregnated with sulphur as soon as the concrete has set sufficiently to allow the ties to be handled without breakage, or if desired, the concrete may be allowed to set until it has reached its maximum strength and then given the sulphur treatment. Hence, either concrete ties which have just been manufactured, or those which are ready to be placed in service, may be advantageously treated with sulphur.

The remarkable increase in tensile strength resulting from the sulphur treatment of the invention has been shown by a series of tensile strength tests which have been conducted for the purpose of comparing untreated and sulphur-impregnated concrete. In carrying out these tests, three sets of tensile briquets were prepared. One of these sets was impregnated with sulphur and tested after a period of 7 days. A second set was impregnated and tested after a period of 28 days, and the third set after a period of three months. In each case unimpregnated control specimens, that is, specimens made of the same proportionate mixture of Portland cement and sand, were broken at the same time with the sulphur-impregnated specimens.

The attached drawings illustrate in detail the remarkable increase in strength imparted to the concrete by the association therewith of sulphur. In these drawings

Fig. 1 is a diagrammatic representation illustrating the results of these tests as shown by the test specimens which were treated and broken at the age of 7 days;

Fig. 2 is a similar strength diagram of specimens treated and broken at the age of 28 days; and

Fig. 3 is a similar diagram of specimens treated and broken at the age of three months.

In each of these figures, curve A shows the tensile strength in pounds per square inch of plain or unimpregnated specimens of concrete containing various percentages of Portland cement. Curve B of each figure shows similarly the tensile strength of correspondingly similar specimens of concrete completely impregnated with sulphur.

In addition to railway ties made of concrete of the usual constituents as just described, railway ties may be made of various other mixtures of materials and then impregnated with sulphur in accordance with the invention. Thus, for example, ties made of a sand-lime mixture such as is now employed for the manufacture of sand-lime brick, or made of a cinder-Portland cement mixture, when impregnated with sulphur

may be used in many instances in place of the concrete tie or the wooden tie. In fact, railway ties may be made in accordance with my present invention from a large number of materials, or combinations of materials which are capable of absorbing molten sulphur and which can be impregnated with molten sulphur. Thus railway ties may be made according to the invention from sulphur-absorbing materials in which the congealed molten sulphur acts as a crystalline binding agent imparting the requisite degree of additional strength and imperviousness to result in a satisfactory and economical tie.

I claim:

1. As an article of manufacture, a railway tie made of relatively soft wood impregnated in part at least with sulphur.

2. As an article of manufacture, a railway tie made of redwood impregnated in part at least with sulphur.

In testimony whereof I affix my signature.

WILLIAM HOFFMAN KOBBE.